

## UNITED STATES PATENT OFFICE

2,078,876

## PRESAPONIFIED BUFFING COMPOUND

Mary F. Hennessey, Waterbury, Conn., assignor to  
The Puritan Manufacturing Company, Water-  
bury, Conn., a corporation of Connecticut

No Drawing. Application October 30, 1936,  
Serial No. 108,471

## 6 Claims. (Cl. 51—280)

This invention relates to abrasive preparations, and more particularly to a solid compound adapted to rub off easily by friction to form a thin coating of abrasive and lubricant upon a revolving buffering wheel for polishing or finishing the surface of a metal or other material.

Every plaster of experience knows the difficulty with ordinary buffering compositions containing free grease when used on pierced, grooved or flared work;—either the work cannot be satisfactorily cleaned and the plate peels, or else the composition will carbonize and must be brushed out of the depressions and holes.

By means of the present invention, the above and other disadvantages have been overcome.

One object of the present invention is to provide a preparation of the above nature containing a binder for the powdered abrasive material, said binder consisting of a presaponified soluble soap made from fatty acids and triethanolamine.

A further object is to provide a buffering compound of the above nature which may be cheaply manufactured in cake form, which will be easy and safe to apply to a buffering wheel either manually or mechanically, which will not rapidly deteriorate in storage, and which will be very efficient in use.

A still further object is to provide a buffering compound of the above nature which will contain no free grease or fat, and may easily be cleaned from the articles after buffering without the use of the strong hot alkali dipping solutions formerly required.

Another object is to provide a buffering compound of the above nature which will be resistant to the carbonizing action of the heat of the buffering operation and in which the water-soluble presaponified binder, as well as the powdered abrasive, will be washed away quickly from the crevices of the buffed articles when dipped in a weak alkali solution without requiring any subsequent brushing or other mechanical operations.

Another object is to provide a buffering compound of the above nature having good detergent, lubricating, abrading and polishing powers, but which will not cause stains, oxidation, tarnishing or discoloration of the work, even upon brass or copper articles.

With these and other objects in view, there have been disclosed in this specification three forms in which the invention may be conveniently embodied in practice.

Three specific examples of the invention will now be described:—

According to the first example, 100 pounds of

oleo-stearine and 20 pounds of double-pressed stearic acid will be placed in a kettle and melted by being brought to a temperature slightly above 130 degrees F.

To this hot mixture, five pounds of triethanolamine  $(C_2H_5OH)_3$  will then be added, and the resultant mixture allowed to stand, while still hot, a sufficient time for thorough commingling and to enable the chemical reaction of saponification to be completed.

The above mixture will then be fed into a suitable mixing machine, which has been previously heated, and there slowly commingled with 220 pounds of tripoli powder and 180 pounds of powdered flint, this mixing operation generally requiring about one and one-half hours. The compound will then be transferred to suitable molds in which it will be allowed to solidify and harden into cakes of suitable size and shape for convenience in application to buffering wheels. The final mixture will have the following proportions:

|                   | Per cent |
|-------------------|----------|
| Oleostearine      | 19.05    |
| Stearic acid      | 3.81     |
| Triethanolamine   | .95      |
| Powdered abrasive | 76.19    |
| Total             | 100.00   |

The presaponified compound of oleostearine, stearic acid and triethanolamine acts as a soluble binder for the abrasive, and causes the latter to stick to the buffering wheel, and lubricate the work during the abrading or polishing process.

The triethanolamine serves to completely saponify the oleostearine and stearic acid, producing a binder for the abrasive having no excess free grease, and resulting in a "soap" having full solubility in water and causing the abrasive particles to quickly wash out of the work after buffering. The work may thus be easily and quickly cleaned by dipping for a short time in a weak solution of alkali at a low temperature, and consequently will not oxidize the metal or produce stains or discoloration on the surface thereof.

In its polishing action, the present buffering compound acts just like any other good composition; i. e. it cuts like the others and colors like them. However, the resemblance stops there, because the present presaponified compound cleans so much better and faster. This is because no time is required for emulsifying and chemically saponifying the greases that are used to bind the particles of abrasive together, as is the case with compositions containing free grease.

*White compound*

According to the second example, 50 pounds of stearic acid will be melted and mixed thoroughly with 37½ pounds of beef tallow. To this mixture will be added two pounds of triethanolamine, and the resultant mass will be allowed to stand till completely commingled and saponified.

While maintaining the above mixture at 130 degrees F., 215 pounds of powdered white silica will then be slowly added, as before, and the compound placed in molds to solidify and harden.

The final mixture will have the following proportions:

|                       | Per cent |
|-----------------------|----------|
| 15 Stearic acid ----- | 16.40    |
| Beef tallow -----     | 12.30    |
| Triethanolamine ----- | .67      |
| White silica -----    | 70.63    |
| 20 Total -----        | 100.00   |

*White stainless compound*

According to the third example, 14 pounds of stearic acid and 9¾ pounds of beef tallow will be melted and commingled thoroughly with two ounces of triethanolamine. After allowing this mixture to stand as before, 72 pounds of white aluminum oxide will be added and thoroughly incorporated in the mixture, which will then have the following proportions:

|                            | Per cent |
|----------------------------|----------|
| Stearic acid -----         | 14.600   |
| Beef tallow -----          | 10.150   |
| 35 Triethanolamine -----   | .013     |
| White aluminum oxide ----- | 75.237   |
| Total -----                | 100.000  |

In use, the end of the bar of buffering compound will be pressed manually or by mechanical means against a revolving buffering wheel of felt, muslin, or other flexible or semi-flexible material. When a sufficient amount of the compound has been deposited on the buffering wheel, the article to be abraded, polished or finished will be held against said wheel until the desired abrading action has been secured. The article may then be thoroughly cleaned by dipping it for a short period of time in hot water or a weak solution of alkali. While triethanolamine has been herein disclosed as the preferred material to be used for saponifying the greases and fatty acids employed in the present buffering compound, it is to be understood that the invention is not limited to this material, but other alkaline materials possessing equivalent mild detergent and emulsification and saponifying properties may also be employed within its spirit and scope. Other such

alkaline materials are the following: monoethanolamine, diethanolamine, ethylene diamine, monoamylamine, diamylamine and triamylamine.

It will also be understood that instead of pre-mixing the greasy material and triethanolamine to form a soap before combining with the powdered abrasive, all three of the essential ingredients may be mixed together simultaneously,—the soap being thus formed during the operation of mixing the other ingredients with an abrasive.

While there have been disclosed in this specification three examples of how the invention may be embodied, it will be understood that the invention is not to be limited to these examples, but may be modified and embodied in various other ways without departing from its spirit. In short, the invention includes all the modifications and embodiments coming within the scope of the following claims.

Having thus fully described the invention, what is claimed as new and for which it is desired to secure Letters Patent, is:

1. A solid abrasive preparation adapted to be deposited by friction upon a revolving buffering wheel comprising a mixture of a fatty acid, triethanolamine, and a powdered abrasive.

2. A solid abrasive preparation adapted to be deposited by friction upon a revolving buffering wheel comprising a mixture of oleostearine 19.05%, stearic acid 3.81%, triethanolamine .95%, and powdered tripoli and flint 76.19%.

3. A solid abrasive preparation adapted to be deposited by friction upon a revolving buffering wheel comprising a mixture of stearic acid 16.40%, beef tallow 12.30%, triethanolamine .67%, and powdered white silica 70.63%.

4. A solid abrasive preparation adapted to be deposited by friction upon a revolving buffering wheel comprising a mixture of stearic acid 14.600%, beef tallow 10.150%, triethanolamine .013%, and white aluminum oxide 75.237%.

5. A solid abrasive preparation adapted to be deposited by friction upon a revolving buffering wheel, comprising a fatty acid presaponified with a substance of the class represented by triethanolamine, monoethanolamine, diethanolamine, ethylene diamine, monoamylamine, diamylamine and triamylamine having mild detergent, emulsifying, and saponifying properties, and mixed with powdered abrasive.

6. A solid abrasive preparation adapted to be deposited by friction upon a revolving buffering wheel, comprising a presaponified compound of a fatty acid and triethanolamine mixed with a powdered abrasive.

MARY F. HENNESSEY.